

## UNITED STATES PATENT OFFICE

2,451,039

## LUBRICANT

Arnold J. Morway, Clark Township, Union County, and John C. Zimmer, Union, N. J., assignors to Standard Oil Development Company, a corporation of Delaware

No Drawing. Application December 27, 1941,  
Serial No. 424,590

5 Claims. (Cl. 252—36)

## 1

The present invention is concerned with the production of improved lubricating grease compositions. The invention more particularly relates to a grease composition which is especially adapted for use under extreme variations in climatic conditions, such as wide variations in temperature and humidity. The preferred composition comprises a mineral oil base thickened to a grease consistency with a mixture of saturated fatty acid soaps of lithium and aluminum.

It is known in the art to prepare various lubricating grease compositions adapted for particular uses. The uses in which grease compositions are employed present a wide variety of conditions and generally a grease prepared with a given set of conditions in mind is not suitable for use under a different set of conditions. Airplanes are controlled in flight by special mechanisms such as rudders, elevators, and ailerons which are attached to the main portions of the airplane such as fuselage and wings by specially designed hinges. These hinges have metal to metal contact bearing surfaces which offer a very difficult lubrication problem. Airplanes are operated under the most severe changes in climatic conditions and since the failure of even one part of the mechanism might well result in a catastrophe, it is imperative that all parts of the plane be maintained in as perfect a mechanical condition as possible. In order to be in good mechanical condition all movable parts should be free and well lubricated at all times. It is not uncommon for a plane during a single trip to be subjected to extremely high ground temperatures, subzero temperatures in the upper atmosphere as well as conditions of high humidity such as rain, snow, or ice. Any lubricant used upon the control mechanisms of the plane must be capable of withstanding these conditions without disintegration.

High temperature greases such as the sodium soap greases are known to the art, however they are quite water-soluble and readily disintegrate under humid conditions. Water - insoluble greases, such as the calcium soap greases, are also known, but these compositions will not withstand high temperatures. Aluminum soap greases are also water insoluble but have a relatively low transient point where they become fluid or rubbery and run or pull out of the bearing.

It is an object of this invention to produce a

## 2

grease composition which will provide adequate lubrication at both high and low temperatures and will not decompose in the presence of excessive moisture. This and other objects will be apparent to those skilled in the art upon reading the following description.

The grease composition made in accordance with the present invention comprises essentially a low pour point lubricating mineral oil distillate, 10 a lithium soap of a saturated fatty acid and an aluminum soap of a saturated fatty acid, although it is preferred to use from 10 to 20% of the lithium soap and from 0.25 to 2% of the aluminum soap based upon the total composition. A small 15 amount of an anti-oxidant, say 0.2%, such as phenyl alpha naphthylamine, may be used if desired.

Although any of the numerous types of low pour point lubricating oils may be used as the 20 base for compositions made in accordance with this invention, it is preferred to use a Coastal type oil having a viscosity, in the range of from about 58 seconds to 100 seconds S. U. V. at 100° F. and a cold test below —40° F.

25 For the formation of the soap utilized in the production of the greases, any saturated fats or saturated fatty acids derived therefrom, such as stearin or stearic acid may be used, although it is preferred to use the saturated acids derived from 30 hydrogenated fish oil.

Any of the methods customarily employed in the compounding of greases may be used in the 35 production of the compositions of this invention. The soaps may be produced separately and then mixed with the oil by heat and agitation; or preferably the saturated fat or fatty acid to be combined with the lithium may be dissolved in a portion of the lubricating oil by heating the oil sufficiently to dissolve the fat or acid in the oil, reacting the fat or fatty acid with lithium hydroxide 40 and then the remainder of the lubricating oil having the aluminum soap dispersed therein may be added after which the mixture is brought to a clear solution and the water driven off by heating 45 and stirring, the anti-oxidant added and the mixture permitted to cool. It is preferred to make the aluminum soap separately and then dissolve it in a portion of the lubricating oil although the aluminum soap can be produced from the saturated fatty acid and aluminum hydroxide in situ

in the oil. Greases of varying consistency to meet the demands of particular conditions may be secured by varying the soap content of the grease within the limits specified. The following examples will serve to illustrate specific embodiments of the invention.

## EXAMPLE 1

|                                               | Percent |
|-----------------------------------------------|---------|
| Hydrogenated fish oil acids                   | 13.00   |
| Lithium hydroxide (monohydrate)               | 2.00    |
| Aluminum stearate                             | 0.50    |
| Lubricating oil (low viscosity, low pour oil) | 42.125  |
| Lubricating oil (low pour Coastal oil)        | 42.125  |
| Phenyl alpha naphthylamine                    | 0.2     |

In compounding the above formula the acid and approximately one-fourth of the oil are charged into a fire-heated kettle equipped with agitators. The mixture is then heated and stirred to a temperature of about 150° F. or until all the acid is melted and dissolved in the oil and then the lithium hydroxide dissolved in boiling water is added to the acid-oil solution. Heating and agitation is continued and the temperature permitted to slowly rise until all of the water is boiled off. During this continued heating small additional amounts of the oil are intermittently added. The aluminum soap is then dissolved in approximately one-fourth of the lubricating oil and this solution together with the remainder of the lubricating oil is added to the kettle after the water has been boiled off. The temperature of the kettle is then raised to within the range of from 350 to 400° F. or preferably about 370° F., at which temperature the grease is completely melted. The phenyl alpha naphthylamine is then added after which agitation and heating is discontinued and the grease permitted to cool forming a smooth almost transparent block. The grease is then worked to a smooth paste in the kettle, filtered and packaged. The grease thus produced has the following characteristics:

|                                          |                |
|------------------------------------------|----------------|
| A. S. T. M. worked penetration at 77° F. | 230            |
| Melting point                            | 374            |
| Free acidity                             | per cent. 0.21 |

<sup>1</sup> Calculated as oleic acid.

Soaking a sample of the grease in water shows no effect on the grease over a period of four weeks. A thin layer of the grease spread out over a steel sheet and subjected to a jet of hot water (175° F.) under force is not washed off, after some 5 hours. No oil separates from the grease after standing for 100 hours at 160° F.

## Low temperature test at -60° F.

Test and apparatus described in paper presented before the 44th annual meeting of the American Society for Testing Materials held in Chicago, Illinois, 6/23-27/41, Performance Specifications for Greases, Robert C. Adams and Harrison E. Patten.

| Force to Turn 3 Bearings Gms. | Approximate Torque Gms.-Cm. | Time for 1 Revolution Secs. |
|-------------------------------|-----------------------------|-----------------------------|
| 300                           | 1,100                       | 95                          |

## EXAMPLE 2

100 parts of hydrogenated fish oil acids are neutralized with 15.73 parts of a lithium hydroxide (monohydrate) dissolved in water. The resulting lithium soap is dried and powdered.

|                                                                                                | Percent |
|------------------------------------------------------------------------------------------------|---------|
| Lithium soap (described above)                                                                 | 15.00   |
| Aluminum stearate                                                                              | 0.60    |
| 10 Phenyl alpha naphthylamine                                                                  | 0.50    |
| Lubricating oil (low pour, Coastal oil < -40° F. pour point, 58 S. S. U. viscosity at 100° F.) | 83.90   |

The lithium soap and aluminum stearate are added to a fire-heated kettle, and one-fourth of the oil added. These ingredients are worked to a smooth paste and the temperature raised to 300° F. The balance of the oil is added and the kettle covered and the temperature raised to 400° F. Stirring and heating is discontinued and the material cooled to room temperature. When cool the solid mass is worked to a smooth plastic homogeneous grease.

The physical properties of this product closely resemble those for the grease described in Example 1.

What is claimed is:

1. An improved lubricating grease composition comprising a major proportion of a low pour point lubricating mineral oil distillate, a minor proportion, sufficient to thicken said oil to a grease consistency, of a lithium soap of a saturated fatty acid and an aluminum soap of a saturated fatty acid, said aluminum soap being present in an amount substantially smaller than that of said lithium soap but not less than 0.25% of the total composition.

2. A composition as defined by claim 1, in which the lithium soap of a saturated fatty acid is the lithium soap of hydrogenated fish oil acids.

3. A composition as defined by claim 1 in which the aluminum soap is aluminum stearate.

4. An improved lubricating grease composition comprising a major proportion of a low pour point lubricating mineral oil distillate, a minor proportion of a lithium soap of a saturated fatty acid amounting to about 10 to 20% of the total composition and a minor proportion of an aluminum soap of a saturated fatty acid amounting to about 0.25 to 1% of the total composition.

5. A composition as defined by claim 1 in which said low pour point mineral oil distillate is a low viscosity distillate.

ARNOLD J. MORWAY.  
JOHN C. ZIMMER.

## REFERENCES CITED

The following references are of record in the file of this patent:

## UNITED STATES PATENTS

| Number    | Name      | Date          |
|-----------|-----------|---------------|
| 1,989,196 | Hilliker  | Jan. 29, 1935 |
| 2,024,990 | Kaufman   | Dec. 17, 1935 |
| 2,066,958 | Brownback | Jan. 5, 1937  |
| 2,186,514 | Yagle     | Jan. 9, 1940  |
| 2,197,433 | Lutz      | Apr. 16, 1940 |
| 2,274,673 | Earle     | Mar. 3, 1942  |
| 2,293,052 | Earle     | Aug. 18, 1942 |